

## UNITED STATES PATENT OFFICE

2,041,635

STEEL FOR RAILROAD RAILS, WHEEL TIRES,  
PLANKPIPES AND OTHER OBJECTS WHICH  
ARE SUBJECTED TO HEAVY WEARHerbert Buchholtz, Dortmund, Germany, assignor  
to firm Vereinigte Stahlwerke Aktiengesell-  
schaft, Dusseldorf, GermanyNo Drawing. Original application December 11,  
1931, Serial No. 580,500. Divided and this ap-  
plication February 13, 1935, Serial No. 6,392.  
In Germany December 12, 1930

2 Claims. (Cl. 75—125)

The invention refers to a further improvement of the steel for railroad rails, wheel tires, plank-piles and other objects which are subjected to heavy wear as claimed and described in my co-pending application Serial No. 580,500 from 5 which the present case is a division.

In said copending application it has been suggested to use for the mentioned purpose a steel containing about 0.05 to 0.2% of carbon, about 0.08 to 0.25% of phosphorus, about 0.1 to 0.6% 10 of silicon, about 0.6 to 1.6% of manganese, about 0.25 to 1% of copper and the balance substantially iron. Now it has been found that by an addition of chromium a further improvement of the wear 15 resistance and the resistance against shock can be obtained. Said improved resistance against shock and impact stresses of a steel containing carbon, phosphorus, silicon, manganese and copper in the proportions above described and in addition thereto from an effective amount to 20 about 1.5% of chromium is especially to be observed with objects of larger extensions. The chromium content is able to improve the notched bar tenacity even in the inner zones of large cross-sections and simultaneously to increase the wear 25 resistance. Thus the addition of chromium is adapted to cause a further improvement of the qualities obtained by the composition described in the copending application. As in my prior 30 composition the sulphur content is preferably kept low so as to lie between a trace and about 0.12%.

The favourable results obtained by the invention are to be seen from the following experiments in which normal carbon steels and those 35 corresponding to my copending application Serial No. 580,500 on the one hand are compared with compositions corresponding to the present invention on the other hand:

| Steel                  | Composition |      |      |       |      |      |
|------------------------|-------------|------|------|-------|------|------|
|                        | C %         | Si % | Mn % | P %   | Cu % | Cr % |
| 1. Normal C-steel..... | 0.38        | 0.10 | 0.73 | 0.080 | 0.02 | ---  |
| 2. P-Mn-steel.....     | 0.15        | 0.20 | 1.45 | 0.090 | 0.25 | ---  |
| 3. P-Mn-Cr-steel.....  | 0.11        | 0.44 | 1.30 | 0.100 | 0.50 | 0.15 |
| 4. P-Mn-Cr-steel.....  | 0.07        | 0.25 | 1.52 | 0.090 | 0.45 | 0.60 |

50 Said steels were subjected to the following tests:

a. In samples of 10 x 10 x 60 mm. with a round notch of a width of 2 mm. and a depth of 5 mm.

the following values have been found for the notched bar tenacity:

|              | Mkg/cm <sup>2</sup> |
|--------------|---------------------|
| Steel 1..... | 3                   |
| Steel 2..... | 10                  |
| Steel 3..... | 10                  |
| Steel 4..... | 11                  |

b. In order to determine the wear on the Spindel-machine the length of the chord was determined as average value obtained with four pieces at a pressure of 5 kg. The total number of revolutions was 250; 25 revolutions were effected per minute. The following values were measured:

|              | Mm. |
|--------------|-----|
| Steel 1..... | 43  |
| Steel 2..... | 41  |
| Steel 3..... | 40  |
| Steel 4..... | 38  |

c. In a further test in order to determine the wear resistance the samples were proved in a machine according to Mohr and Federhaff. The samples were subjected to 200,000 revolutions performed at a pressure of 100 kg., 1% sliding; 425 revolutions were performed per minute. The following values were found for the loss in weight:

|              | Grms. |
|--------------|-------|
| Steel 1..... | 1.4   |
| Steel 2..... | 1.0   |
| Steel 3..... | 0.9   |
| Steel 4..... | 0.8   |

What I claim and desire to secure by Letters Patent of the United States of America is:

1. A steel for railroad rails, wheel tires, plank-piles and other objects which are subjected to heavy wear, said steel containing about 0.05 to 0.20% of carbon, about 0.08 to 0.25% of phosphorus, about 0.1 to 0.6% of silicon, about 0.6 to 1.6% of manganese, from an effective amount to about 1.5% of chromium and about 0.25 to 1% of copper and the balance substantially iron.

2. A steel for railroad rails, wheel tires, plank-piles and other objects, which are subjected to heavy wear, with a sulphur content of from trace to about 0.12%, said steel containing about 0.05 to 0.20% of carbon, about 0.08 to 0.25% phosphorus, about 0.1 to 0.6% of silicon, about 0.6 to 1.6% of manganese, from an effective amount to about 1.5% of chromium and about 0.25 to 1% of copper, and the balance substantially iron.

HERBERT BUCHHOLTZ.